

T. F. TESSE.

PROCESS FOR DIMINISHING THE VISIBILITY OF OBJECTS.

APPLICATION FILED JUNE 24, 1918.

1,426,521.

Patented Aug. 22, 1922.

Fig. 1.



SOLID ARTICLE, SHIP OR LIKE.



Fig. 2.

WITNESSES

J. H. Crawford  
A. B. Foster

INVENTOR

J. F. Tesse  
BY  
Ken. Page, Cooper & Hayward  
ATTORNEYS

# UNITED STATES PATENT OFFICE.

THEODORE FRANÇOIS TESSE, OF ST.-OUEEN, FRANCE, ASSIGNOR TO SOCIETE NAUTON FRERES & DE MARSAC, OF ST.-OUEEN, SEINE, FRANCE, AND THEODORE FRANÇOIS TESSE, OF PARIS, FRANCE.

## PROCESS FOR DIMINISHING THE VISIBILITY OF OBJECTS.

1,426,521.

Specification of Letters Patent. Patented Aug. 22, 1922.

Application filed June 24, 1918. Serial No. 241,685.

To all whom it may concern:

Be it known that I, THEODORE FRANÇOIS TESSE, of No. 15 Rue des Rosiers, Saint-Ouen, Seine, France, have invented an Improved Process for Diminishing the Visibility of Objects, of which the following is a full, clear, and exact description.

This invention has for its object to provide an improved process for diminishing the visibility of objects, and more particularly the visibility of aeroplanes, seaplanes, ships, etc., for the purpose of rendering it difficult for such objects to be seen and located at night by means of searchlights.

15 The improved process consists essentially in producing upon the object upon which the light beam is projected, a progressive extinction of the differently coloured rays constituting the said beam.

20 This result is effected by providing the object with two or more coats of varnish of different natures, namely, a first coat applied directly upon the object, and composed of a very opaque varnish or composition having a matte surface and a very dark colour in which black or blue predominates. Upon this first coat, one or more other coats are applied, composed of a translucent coloured varnish, the colour of

25 which is chosen according to the nature of the source of light, in such a manner as to arrest the greater part of the rays of a projected light beam striking the object.

30 This combination has the effect that when 35 a beam of light is thrown upon an object covered with the above stated various coats of varnish or composition, a great part of the rays of which the light beam is composed is first of all arrested by the coat of transparent varnish, acting as a screen.

35 Then the remainder of the light which has passed through said transparent coloured varnish is finally absorbed by the dark coloured matte opaque coat. In these circumstances the proportion of the light rays that is reflected by the object is practically nil, and consequently the visibility of said object is thereby rendered very low.

The composition of the transparent var-

nish and of the opaque varnish will vary 50 according to the predominant colour in the projected rays of light.

The first coat, that is to say, that which is applied directly to the object, must contain opaque pigments having a very great 55 light absorbing capacity. This first coat may consist for instance of lamp black incorporated in a vehicle or medium such as a fatty varnish, a coating composition of cellulose acetate, insoluble gelatine, etc. To 60 this lamp black there may be added an opaque colouring matter such as Paris blue, ochres, sienna earth, etc.

The outer coat consists of a red lake 65 preferably a red lake having a bluish ground, that is to say, having a violet-tinted colour when it is viewed by transmitted light. It has been found by experience that red colour, and particularly the 70 red colouring matters of aniline have the power of absorbing the greater part of the rays emitted by the sources of light that are usually employed, i. e., an ordinary searchlight. An exception must however be made 75 in the case of the fluorescent aniline colouring matters of the triphenylmethane group which are derived from phthalic acid (eosines, rhodamines), these colouring matters having the property of gleaming or 80 sparkling with a great brilliance in the dark when illuminated by light containing violet rays. These colours are accordingly not used.

For colouring this transparent coat it is preferred to employ the red colouring matters of alizarine acid which are derivatives 85 of anthranilic acid converted into barytic lakes or others, and precipitated upon pure uncalcined hydrate of alumina.

For constituting the coloured coats applied in the improved process, use may be made of all coloured or colouring products of any kind, paints, fatty varnishes, celluloid, cellulose esters, insoluble gelatine, and especially cellulose esters, etc.

In applying the improved process to the aeroplane fabrics it is preferred to employ coloured coating composition having a base

of cellulose acetate, also containing as specified in my earlier patent application filed January 10, 1916, Serial No. 71,201, the following essential substances:

5 a—a dilute solution of cellulose acetate in methyl acetate or acetone solvent, for instance in the proportion of 7 to 8%.

b—a high boiling point solvent in a proportion of approximately 2%. This solvent 10 should be one capable of completely evaporating, such as benzyl alcohol or aceto-acetic ether, whose function is to serve solely as an antiroughening agent and facilitate the proper formation of the coating skin.

15 c—a softening body such as tri-acetin, in small amount, for instance 0.5 to 1%.

d—a solvent having a very high boiling point, in the proportion of for instance 20 about 2%. This should be one which does not evaporate during the process, such as eugenol or isoeugenol, which has the function of increasing the plasticity of the composition, and is itself capable of undergoing 25 certain transformations by way of polymerisation.

e—inert coloured matters (or pigments) serving as the tensioning agent in the very flexible coating skin thus produced; said 30 inert coloured matters being employed in the proportion of about 1 to 3%. As examples of such pigments, lamp black or Paris blue are mentioned.

As specified in the earlier Patent application 35 of the present applicant 123,640 filed October 4, 1916, this flexible coating skin which is composed of the above specified substances, is imprisoned between two relatively non-plastic rigid coats of composition, 40 such for example as cellulose acetate.

I have now described by way of example a manner of carrying out the improved process in its application for coating aeroplane fabrics and preventing their visibility 45 when they are illuminated by searchlights in the dark.

This practical example consists in applying successively the following coats:

1.—A rigid non-plastic coat of cellulose 50 acetate which does not contain inert substances, and which has a tensioning effect upon the fabric (e. g., cellulose acetate alone).

2.—A coat having a matte and dark- 55 coloured coat, having an opaque ground consisting of a flexible composition composed of the substances specified above under a, b, c, d and e, in which black or blue pigments such as lamp black, Paris blue (or 60 a plurality of such), are employed as the inert ingredients.

3.—A transparent coat likewise consisting of a flexible composition composed of the same substances as specified under a, b, 65 c, d and e, but wherein the inert ingredient

is constituted by a lake of alizarin red, or any other similar lake which is very rich in colouring matter, precipitated upon hydrate of alumina and containing no mineral loading material whatever. The lake and the hydrate of alumina must be very pure in order that the coat shall be highly transparent.

4.—A coat of a tensioning rigid composition which does not contain any inert matter, and is similar to the composition constituting the first coat.

When the process is applied to objects besides aeroplane fabrics, such as for instance to vessels, any suitable paints may 80 be employed which are capable of producing by their superposition the above defined optical effect. In such a case the coats that are employed need not have the plastic and tensioning properties which are necessary 85 for treating aeroplane fabrics.

The improved process may also be carried out by the application of a number of successive coats of monochromatic transparent varnishes of different colours, capable 90 of absorbing respectively the various rays of different colours of which the projected beam of light is composed.

It is to be understood that the composition of the coats and their colouring may vary 95 according to the applications, the nature of the objects, and the nature of the source of the projected light.

The accompanying drawing shows two of the various forms of coatings embraced 100 within the scope of the present invention, the figures being exaggerated sections.

Fig. 1 shows an aeroplane wing fabric impregnated and coated with cellulose acetate, then having a layer of a first coating, 105 then a layer of a second composition, and then another layer of cellulose acetate.

Fig. 2 shows a solid article, such as a ship, with a two-layer coating forming a simple example of the present invention.

I claim:

1. A process for diminishing the visibility of objects and preventing their being picked up by an artificial beam of light, consisting in applying a first coat, called ground coat, 115 composed of an opaque varnish or composition having a matte surface and a dark colour and then a transparent or translucent coloured varnish, the colour of which bears such a relation to that of the ground coat 120 and to the character of the artificial beam of light, that the greater part of the rays of the projected light beam will be arrested and a product of low visibility produced.

2. A process for diminishing the visibility 125 of objects and preventing their being picked up by an artificial beam of light, consisting in applying a ground coat composed of dark coloured opaque pigments, of blue to black shades, incorporated in a vehicle capable of 130

producing a film-coating; and then applying a transparent coat carrying a red lake, the colors of such two coats being such as to substantially lower the visibility of the object coated.

3. A process for diminishing the visibility of objects and preventing their being picked up by an artificial beam of light, consisting in applying a ground coat composed of dark 10 coloured opaque blue-to-black pigments, incorporated in a vehicle including a cellulose ester and solvents therefor, and then applying a transparent coat carrying a red lake of alizarin precipitated upon pure hydrate 15 of alumina.

4. A process for coating aeroplane fabrics and preventing their visibility when they are struck at night by the beam of light of a searchlight, consisting in applying a dark 20 coloured, matte, opaque coating having a basis of cellulose acetate and containing a coloured inert substance producing a tensioning effect, and in thereafter applying a transparent coating also having a basis of cellulose acetate, containing an inert 25 substance producing a tensioning effect and comprising a red alizarin lake precipitated upon pure hydrate of alumina.

5. A process for coating aeroplane fabrics 30 and preventing their visibility when they are struck at night by the beam of light of a searchlight, consisting in applying a dark coloured, matte, opaque coating having a basis of cellulose acetate, and containing a dark 35 blue-to-black coloured inert substance producing a tensioning effect; and in then applying a transparent coating having also a basis of cellulose acetate and containing an inert substance producing a tensioning 40 effect and comprising a red alizarin lake precipitated upon pure hydrate of alumina; each of the coloured and respectively opaque and transparent coatings being composed of a dilute solution of cellulose acetate in a volatile solvent thereof, a solvent having a 45 higher boiling point, serving as an anti-roughening agent, a softening substance, and a solvent having a very high boiling point also serving as plasticifying agent.

6. A process for coating aeroplane fabrics 50 and preventing their visibility when they are struck at night by the beam of light of a searchlight, consisting in applying a dark coloured, matte, opaque coating having a basis of cellulose acetate and containing a dark 55 blue-to-black coloured inert substance producing a tensioning effect; and in then applying a transparent coating having also a basis of cellulose acetate and containing an inert substance producing a tensioning effect 60 and substance comprising a red alizarin lake precipitated upon pure hydrate of alumina, each of these coloured and respectively opaque coats being applied between two 65 substantially rigid non-plastic coats.

7. A process for diminishing the visibility of objects and preventing their being picked up by an artificial beam of light, consisting in applying a first coat composed of a dark coloured, matte, opaque coating composition; 70 then a plurality of successive coats of coating compositions which are transparent or translucent, monochromatic, differently coloured, and capable of absorbing respectively the various rays constituting the beam 75 of light.

8. A coated article of low visibility, such article having a coating carrying dark blue-to-black pigment and having a matte surface, and a superposed coating carrying a red 80 lake, the colors of such coatings being so related as to produce a lowered visibility in the article, as compared with the same article having the same first coating only.

9. A coated article possessing low visibility 85 comprising an article having a ground coating composed of dark colored matte opaque blue-to-black pigments incorporated in a vehicle including a cellulose ester and a substantially non-volatile liquid solvent and a plasticifying agent; and a superposed transparent to translucent coating comprising a red alizarin lake precipitated upon hydrate of alumina, carried in a cellulose ester. 90

10. A coated aeroplane fabric of low visibility 95 comprising a fabric carrying a dark colored matte opaque coating having a basis of cellulose acetate and containing a dark blue-to-black pigment capable of producing a tensioning effect; and a superposed transparent to translucent coating having a basis of cellulose acetate and containing an inert 100 material capable of producing a tensioning effect and comprising a red alizarin lake precipitated upon hydrate of alumina. 105

11. A coated aeroplane fabric of low visibility comprising a fabric carrying a dark colored matte opaque coating having a basis of cellulose acetate and containing a dark blue-to-black pigment capable of producing 110 a tensioning effect; and a superposed transparent to translucent coating having a basis of cellulose acetate and containing an inert material capable of producing a tensioning effect and comprising a red alizarin lake precipitated upon hydrate of alumina, said two 115 coatings being imprisoned between films of cellulose acetate.

12. A coated aeroplane fabric of low visibility comprising a fabric carrying a dark 120 colored matte opaque coating having a basis of cellulose acetate and containing a dark blue-to-black pigment capable of producing a tensioning effect, together with a substantially non-volatile solvent capable of serving 125 as an anti-roughening agent, a softening substance and a plasticifying agent; and a superposed transparent to translucent coating having a basis of cellulose acetate and containing an inert material capable of pro- 130

ducing a tensioning effect and comprising a red alizarin lake precipitated upon hydrate of alumina.

13. A coated aeroplane fabric comprising  
5 a fabric base, a coating composed of a dark  
colored, matte, opaque coating composition;  
and a plurality of successive superposed  
coats of transparent to translucent mono-  
chromatic, differently colored coating com-

positions, which are capable of absorbing 10  
respectively the various rays of which a  
beam of light is composed.

Signed by me, this 23rd day of May, 1918.

THEODORE FRANÇOIS TESSE.

Witnesses:

CHAS. P. PRESSLY,  
EMILE BERTRAND.